

# United States Patent

[11] 3,561,638

[72] Inventor **Jean B. Morjan**  
Koekelberg-Brussels, Belgium  
[21] Appl. No. **755,209**  
[22] Filed **Aug. 26, 1968**  
[45] Patented **Feb. 9, 1971**  
[73] Assignee **Etablissements J. B. Gabriels S.P.R.L.**  
Koekelberg-Brussels, Belgium  
a company of Belgium  
[32] Priority **June 14, 1968**  
[33] **Belgium**  
[31] **48,034**

[56] **References Cited**  
UNITED STATES PATENTS  
3,102,831 9/1963 Tisdale ..... 75/123J  
3,257,200 6/1966 Hodge ..... 75/123J  
FOREIGN PATENTS  
685,397 4/1964 Canada ..... 75/123J  
*Primary Examiner—Winston A. Douglas*  
*Assistant Examiner—A. Skapars*  
*Attorney—Richards and Geier*

[54] **BOX OR CONTAINER OF METAL SHEET HAVING  
A SMALL THICKNESS AND BEING SUBJECTED  
TO HIGH INTERNAL PRESSURES**  
5 Claims, 2 Drawing Figs.

[52] **U.S. Cl.** ..... **220/67,**  
148/34  
[51] **Int. Cl.** ..... **B65d 7/42**  
[50] **Field of Search** ..... 148/34, 31,  
39; 75/123J, 124; 220/67, 3, 24, 1, 83; 29/186

**ABSTRACT:** This invention relates to boxes or containers of metal sheet having a small thickness and being provided for storage and distribution of beers and other drinks rich in carbonic gas under pressure, with ends made of rolled sheet having a high yield strength of soft steel recrystallized by annealing and the composition of which contains Nb in the range of 0.015 percent to 0.050 percent by weight of the composition.

PATENTED FEB 9 1971

3,561,638

FIG. 1  
FIG. 2



INVENTOR.  
BY Jean B. Morjan  
Richards & Geier  
ATTORNEYS

**BOX OR CONTAINER OF METAL SHEET HAVING A  
SMALL THICKNESS AND BEING SUBJECTED TO HIGH  
INTERNAL PRESSURES**

This invention relates to boxes or containers of metal sheet having a small thickness and being constructed for storage and distribution of beers and other drinks rich in carbonic gas under pressure.

The distribution under pressure requires the use of containers having a capacity substantially larger than the conventional storage box. For instance, a container has a height of approximately 225 mm. and a diameter of approximately 155 mm., namely a capacity of approximately 4 liters. Under an equal pressure, the stress exerted upon the walls of the container is thus much more important than in the conventional storage box the capacity of which does not generally exceed 1 liter.

The initial pressure being already relatively high, it follows that any increase of the room temperature causes a substantial increase of the internal pressure. This problem is still more important in that the metallic containers or boxes according to the present invention must be capable of withstanding internal pressures resulting, e.g., from the pasteurization temperature, namely about 60 to 65°C. In addition, such temperatures may be generally reached incidentally, namely when the containers are housed in relatively overheated rooms or locations.

Temperatures between 50 and 60°C. have been observed in the motor car trunks, as well as in rooms the windows of which are facing south, the panes forming true lenses concentrating the sun rays upon the metallic boxes and the like.

Generally, by the conventional technical means and compositions and for acceptable thicknesses of approximately 0.32 mm. for the body of the container and 0.60 mm. for the ends, a satisfactory resistance may be only obtained for internal pressures which do not exceed 4 kg/cm<sup>2</sup>.

Of course, the use of heavier sheets could be suggested as a solution. Unfortunately, such solution would be unacceptable for both economical and technical reasons. In fact, it is apparent that owing to the industrial production means, the raw material has a substantial influence upon the cost price of such metallic boxes or containers. In addition, it must be also taken into consideration that, owing to the production rate, the tools and the good preservation of the industrial equipment, some sheet thicknesses must not be exceeded.

From the above considerations, it results that neither the steel compositions nor the production means known heretofore allow to manufacture, within the minimum thicknesses generally used, a metallic box or container having a sufficient resistance for the storage and the distribution of beer under pressure with all the safety conditions required by the brewery and without requiring the storage in a refrigerator.

While the manufacture of the body of such cylindrical boxes in tinned sheet with a thickness of approximately 0.32 mm. does not set any problem, the resistance being sufficient, the same is not true for the ends, owing to their proper morphology constituting the weak points of the container, since it is well known that any excess of internal pressure causes the bulging thereof, with, consequently, a deterioration of the crimping and other known consequences such as leakages, alteration of the content and the like.

On the other hand, it is not possible to substantially increase the thicknesses of the ends owing to the requirements of the manufacture itself and also for economic reasons. It results that, in the present state of the industry, it is not possible to find, in the conventional grades generally used in the industry for the manufacture of metallic storage containers, sheets suitable for the rational manufacture of ends for containers which must withstand the previously mentioned pressures.

Nevertheless, the object of the present invention is to allow the industrial manufacture, with the normal tools and equipments, of such metallic boxes having a capacity of approximately 4 litres under perfectly acceptable economic conditions, the cost prices being very near the prices resulting from the use of the conventional sheets although the containers have a substantially increased resistance.

Two metallic containers embodying the present invention are hereinafter described with reference to the appended drawings, wherein:

FIG. 1 is an exploded view, in cross section of the three parts of the container;

FIG. 2 is partly an elevational view of and partly a section through the container of FIG. 1, after assembly.

In these FIGS., 1 shows the body of the container, in this instance cylindrical; 2 and 3 designate the ends with which the present invention is particularly concerned.

According to the invention, this resistance increase is obtained, not by the increase of the thickness of the sheets used for the manufacture of the ends, but manufacture a substantial increase of the yield strength of such sheets.

This seems to be simple, but sets truly problems which have appeared to be very difficult to solve, on one hand because it is not known to manufacture tinned sheets which, after rolling and annealing, have both a high yield strength of about 40 Kg./mm.<sup>2</sup> and sufficient crimping possibilities to allow the manufacture of boxes with the known tools and techniques and, on the other hand, because the addition of hardening elements to steel in the proportions necessary for obtaining such high yield strength is not compatible with the requirements relating to the storage of foods and more particularly to beer.

In fact, it is known that the corrosion of a can by the foods contained therein depends not only upon the quality and the thickness of the tin layer, but also upon the composition and the nature of the supporting sheet.

According to the practice defined by national and international standards, the sheet for storage is essentially a sheet made from an effervescent soft steel in the composition of which are prohibited or at least limited the hardening elements promoting the corrosion such as Si, C, Mn, P, N, A1 and Cu are admitted, but they do not allow to reach, in the finished products, a high yield strength together with a sufficient elongation. There are also sheets in which a high yield strength is obtained by postrolling after annealing, but to the prejudice of the elongation which becomes quite insufficient. (See, e.g., the sheet described in the German Pat. No. 1,247,362 which, for a yield strength of 44.4 kg/mm.<sup>2</sup>, has only an elongation of 10 percent upon a sample of 5.08 cm.).

According to the principal object of the invention, for realizing ends for the industrial manufacturer of metallic boxes or containers being pressurized and more particularly of such metallic cylindrical boxes or containers having crimped ends and a capacity of approximately 3 to 4 litres for containing a liquid under pressure, generally beer, there is used a cold rolled sheet recrystallized by annealing in the top hat furnace and having a minimum yield strength of 40 kg. and a minimum elongation of 20 percent, said sheet being manufactured from a killed steel containing, in addition to moderate proportions of ordinary hardening elements such as C, Si and Mn, a sufficient amount of Nb to reach the said level of yield strength in the cold rolled and annealed product, the use of said sheet being combined with the use of a protecting varnish.

It is apparent that, for solving the specific problems set forth, the invention used simultaneously three means, namely: reducing the extent of hardening additions detrimental for

corrosion; increasing, by substantial addition of Nb, the yield strength after cold rolling and annealing, while maintaining sufficient crimping possibilities; and completing the corrosion resistance by the use of a layer of protecting varnish.

According to the invention, the steel composition meets the following analysis:

P 0.040 percent maximum

Mn 0.650 to 0.950 percent

C 0.060 to 0.100 percent

Si 0.200 to 0.400 percent

A1 0.020 percent minimum

Nb about 0.020 percent, between 0.010 and 0.030 percent maximum.

Those skilled in the art will very readily conform to the level of the yield strength and the elongation by varying these elements within the specified limits.

On the basis of the principle of equivalents, the invention claims also the replacement of Nb by elements which, like the latter, are likely to induce a structural hardening by the formation of carbides, nitrides or nitrocarbides. Nb has been specifically selected since it is the cheapest element being used very readily.

It has been established that cylindrical metallic boxes being 225 mm. in height and 155 mm. in diameter; i.e. boxes having a capacity of approximately 4.25 litres, the body being made of a tinned sheet having a thickness of 0.32 mm. and the ends being made of a steel sheet of the previously mentioned composition and being 0.60 mm. in thickness, have had very good resistance to an extraordinary internal pressure of approximately 6 kg./cm.<sup>2</sup> without any detrimental deformation, the said metallic boxes being subjected to a temperature of approximately 60° C. The experimented containers contained beer under a CO<sub>2</sub> pressure. When the container and content thereof have been brought back to room temperature, it has been possible to distribute beer under pressure in absolutely normal conditions up to the complete emptying. Such experiments repeated several hundred of times have all confirmed such results.

In this nonlimitative example, the analysis of the sheet was as follows:

|    |               |
|----|---------------|
| P  | 0.028 percent |
| Mn | 0.85 percent  |
| S  | 0.030 percent |
| C  | 0.082 percent |
| Si | 0.320 percent |
| A1 | 0.059 percent |
| Nb | 0.026 percent |

The tinned sheet had the following characteristics:

Yield strength: 41.7 kg./mm.<sup>2</sup>

Break load: 53.2 kg./mm.<sup>2</sup>

Elongation: 24.4 percent

R30 hardness: 69

Erickson: 8.4

It is apparent that the elongation and the Erickson's value are substantially higher than of known tinmed sheets having the same yield strength (namely the "Temper 6" of the American Classification).

I claim:

1. A metallic box or container made of a sheet having a small thickness and being subjected to high internal pressures, characterized in having two ends made from a cold rolled soft steel sheet having a yield strength higher than 35 kg./mm.<sup>2</sup> and an elongation higher than 20 percent, recrystallized by annealing and the composition of which contains, in addition to the usual hardening elements an amount of Nb in the range of 0.015 percent to 0.050 percent by weight of the composition.

15 2. A metallic box or container according to claim 1, characterized in that the recrystallization annealing after cold rolling of the sheet used for making both ends is effected in a top hat furnace.

3. A metallic box or container according to claim 1, characterized in that the steel used for making both ends consists of a carbon steel which is manufactured according to the conventional methods of hot rolling, cold rolling, annealing and skin-pass, the recrystallization annealing after cold rolling being effected in a top hat furnace.

25 4. A metallic box or container according to claim 1, characterized in that both ends are made from a cold rolled sheet having a composition within the following limits, by weight of the composition which additionally includes:

|    |                        |
|----|------------------------|
| P  | 0.040 percent maximum  |
| Mn | 0.500 to 1.500 percent |
| C  | 0.050 to 0.200 percent |
| S  | 0.030 percent          |
| Si | 0.250 to 0.400 percent |
| A1 | 0.040 to 0.100 percent |
| Cu | 0 to 0.400 percent     |

35 5. A metallic box or container according to claim 1, characterized in that the internal walls are covered with a protecting layer of varnish.